

## 1

3,268,421

ELECTRODEPOSITION OF METALS FROM A  
FUSED BATH OF ALUMINUM HALOHY-  
DRIDE ORGANIC COMPLEX AND COMPO-  
SITION THEREFOR

Leslie D. McGraw, Columbus, Ohio, assignor, by mesne assignments, to National Steel Corporation, Pittsburgh, Pa., a corporation of Delaware  
No Drawing. Filed Dec. 4, 1961, Ser. No. 156,966  
25 Claims. (Cl. 204—39)

This invention broadly relates to the electrodeposition of metals and, in some of its more specific variants, to novel compositions useful as baths for the electrodeposition of metals and to a process for electrodepositing metals therefrom. The invention further relates to a process for preparing the baths of the invention, additives therefor, and a new chemical compound.

The invention may be illustrated and described hereinafter with specific reference to the electrodeposition of aluminum on a conductive substrate employing the novel baths of the invention. However, it is understood that the invention is not limited thereto and that aluminum alloys, or still other metals or metal alloys may be electrodeposited from the novel plating baths of the invention.

A number of processes have been proposed heretofore for the electrodeposition of aluminum. For instance, aluminum may be electrodeposited from fused inorganic salt baths containing at least 75% by weight aluminum chloride and the remainder alkali metal chloride, or from prior art organic baths comprising a solution of an aluminum salt in a highly inflammable organic solvent such as ethyl ether. While satisfactory aluminum electrodeposits may be obtained from the foregoing baths, they each have objectionable features. For instance, the inorganic bath fumes excessively at the relatively high operating temperature and some means must be provided for controlling the fuming. The organic baths of the prior art do not present a fuming problem but the organic solvent is inflammable and presents a serious fire hazard at the operating temperature. As a result, there has long been a need for a satisfactory bath for the electrodeposition of aluminum which does not present the fuming problem of the inorganic baths and which is noncombustible at the operating temperature.

It is an object of the present invention to provide a novel composition of matter which is especially useful as a bath for the electrodeposition of metals or metal alloys.

It is a further object to provide a novel plating bath for electroplating aluminum on a conductive substrate.

It is still a further object to provide additives for the baths of the invention whereby the initial resistivity may be reduced.

It is still a further object to provide the new chemical compound ethoxyethyltrimethyl ammonium chloride.

It is still a further object to provide a novel process for the electrodeposition of metals and metal alloys from the baths of the invention.

It is still a further object to provide a novel process for electroplating aluminum on a conductive substrate from the novel plating baths of the invention.

It is still a further object to provide a novel process for preparing the plating baths of the invention.

Still other objects and advantages of the invention will be apparent to those skilled in the art upon reference to the following detailed description and the specific examples.

In accordance with one variant of the present invention, novel compositions of matter are provided which consist essentially of an organic complex of an aluminum halo hydride, with or without an organic complex of an aluminum halide. The resultant compositions are

## 2

useful for the deposition of metal on a substrate, and they are especially useful as a bath in the novel process of the invention for the electrodeposition of a metallic material on a conductive substrate.

5 In accordance with a more specific variant of the invention, novel baths are provided for the electrodeposition of a metallic material on a conductive substrate which consist essentially of an etherate of an aluminum halo hydride, with or without an etherate of aluminum halide. 10 The resultant baths are noncombustible at the operating temperature, i.e., the temperature at which the metallic material may be electrodeposited on the substrate. Preferably, the metallic material comprises aluminum.

The aluminum halo hydrides suitable for practicing 15 the present invention may include complexes of compounds of the general formula  $AlH_mX_n$ , where X is halogen, m and n each have a numerical value of at least one, and  $m+n$  are equal to three. Thus, in the foregoing general formula the atomic ratio of Al to H is between 1:1 and 1:2, the atomic ratio of Al to X is between 1:2 and 1:1, and the atomic ratio of Al to  $H+X$  is 1:3. Specific 20 examples of aluminum halo hydrides includes  $AlHX_2$ ,  $AlH_2X$ , and mixtures thereof such as  $Al_3H_4X_5$ , which may be written as  $AlH_{4/3}X_{5/3}$  for the purpose of this discussion. Chlorine and bromine are preferred over other halogens in most instances.

25 Preferably the foregoing aluminum halo hydrides are present in the form of coordinate covalent complexes. The complexes may be prepared by reacting the aluminum halo hydride with one or a mixture of compounds which are known to be complexing agents therefor and especially Lewis bases such as ethers, or suitable compounds in general containing a functional group which is capable of complexing aluminum halo hydride and/or aluminum halide, such as organic compounds containing a divalent sulfur atom including the thioethers, organic compounds containing a trivalent nitrogen atom such as the amines, and organic compounds containing a trivalent phosphorus atom. An ether or a mixture of ethers is usually preferred as the complexing agent. A wide variety of ethers may be employed in forming the resultant etherate such as ethyl ether, propyl ether, butyl ether, octyl ether, etc., and ethers in general wherein the organic groups attached to the oxygen atom contain, for example, about 1 to 8-20 carbon atoms. The ether may contain an aromatic group such as methylphenyl ether, ethylphenyl ether, diphenyl ether, etc., or a cyclohydrocarbon radical and especially those containing carbon atoms within the foregoing ranges. Ethers containing a plurality of ether linkages and organic radicals as above discussed or their equivalents also may be used, such as diethylene glycol diethyl ether, or cyclic ethers such as tetrahydrofuran. Diethyl ether or a mixture of ethers comprising diethyl ether is usually preferred.

30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420

dry inert gas to an extent to render the resultant composition noncombustible at the operating temperature of a bath prepared therefrom. Usually, it is more convenient to prepare an aluminum halohydride-containing complex by dissolving aluminum halide in a solvent, adding the complexing agent and an active hydrogen-containing compound to the solution in an amount to provide the desired amount of active hydrogen in the resultant composition, and reacting the mixture to produce a complex of aluminum halohydride. In instances where the aluminum halide is present in excess, a mixture of the complexes of aluminum halohydride and aluminum halide is produced. The solvent and complexing agent may be the same substance, such as when an ether is used as the solvent and complexing agent. The solvent may be removed subsequent to the reaction as noted above and the reaction product used in preparing the baths of the invention.

When an etherate of an aluminum halohydride is prepared, preferably aluminum halide is dissolved in an excess of diethyl ether and then one or a mixture of metal hydrides such as aluminum hydride, alkali metal hydrides such as sodium, potassium or lithium aluminum hydride, or alkaline earth metal hydrides such as calcium hydride, is added to the solution in the calculated quantity to provide the desired amount of active hydrogen in the resultant composition. The metal hydride may be added in the calculated amount to react with the aluminum halide and produce a desired aluminum halohydride etherate, or in a smaller amount so as to have the aluminum halohydride etherate present in solution together with aluminum chloride etherate. When metal hydride is reacted with aluminum halide, preferably the mole ratio of aluminum hydride ( $\text{AlH}_3$ ) to aluminum halide ( $\text{AlX}_3$ ) in the resultant aluminum halohydride-containing composition is between 1:0.5 and 1:22, and for better results between 1:2 and 1:11. In the present specification and including the claims, for convenience the mole ratio of aluminum hydride ( $\text{AlH}_3$ ) to aluminum halide ( $\text{AlX}_3$ ) in the aluminum halohydride-containing bath compositions of the invention is calculated by considering the aluminum halohydride content to be a mixture of  $\text{AlH}_3$  and  $\text{AlX}_3$ , and free aluminum halide, if any, is added thereto. For example, a bath composition containing only three moles of an etherate of  $\text{AlHCl}_2$  would contain one mole of  $\text{AlH}_3$  for each of two moles of  $\text{AlCl}_3$  and the  $\text{AlH}_3$  to  $\text{AlCl}_3$  ratio would be 1:2. If the bath also contained one mole of an etherate of free aluminum chloride for each three moles of  $\text{AlHCl}_2$ , then the  $\text{AlH}_3$  to  $\text{AlCl}_3$  ratio would be 1:3 due to the presence of the excess aluminum chloride.

After reaction of the metal hydride with the ether solution of aluminum halide, the excess ether over that required to form the etherate may be evaporated by heating and/or by aeration with a dry inert gas. The ether solution often may be merely heated to its boiling point and the free or solvent ether boiled off. When this is done, the boiling point of the resultant composition rises slowly with evaporation of ether until the monoetherate of the aluminum halohydride and aluminum halide is formed. When diethyl ether is used as the solvent, the flash point of the resultant composition will rise to about 200-215° F. and there is no further appreciable rise. The resultant composition is noncombustible and may be decanted and used as a plating bath. When the ether is diethyl ether, preferably the solvent ether is removed by boiling the solution until the boiling point rises to about 150-160° F. Then, a dry inert gas such as nitrogen, helium, argon, etc., is passed through the composition at a lower temperature such as 90° F. for the purpose of removing an additional amount of solvent ether and raising the flash point up to about 200-215° F. This latter procedure has the advantage of reducing thermal decomposition and thermal decomposition may be further reduced by using only aeration with dry, inert gas at temperatures

of 70-90° F. for removing the solvent. Anhydrous conditions should be maintained throughout the reaction and during the removal of excess ether for the purpose of preventing decomposition of the aluminum halohydride.

The plating baths of the present invention preferably are treated to remove organic solvent until the vapor phase is in equilibrium with the bath at the operating temperature is nonexplosive and noncombustible in air. When diethyl ether is the solvent, the ether content of the vapor phase should not be greater than about 1% by volume in most instances. The ether content that remains is largely combined chemically with the aluminum halohydride and aluminum chloride in the form of etherates. The etherates are stable at the operating temperature of the bath, and thus ether is not available in the free or uncombined form for forming a combustible or explosive mixture. The resultant noncombustible aluminum halohydride-containing compositions may be used in preparing baths for the electro-deposition of a metal such as aluminum or aluminum alloys.

The thermal stability of the bath is often improved when excess or free aluminum halide complex is present. Usually, the mole ratio of  $\text{AlH}_3$  to  $\text{AlCl}_3$  should not be higher than about 1:3, and preferably not higher than about 1:6. The bath should be at least 1 molar in active hydrogen, i.e., at least one molar in  $\text{AlHCl}_2$  or the equivalent in active hydrogen content. The plating baths of the invention generally may be used at temperatures above the melting point and below the decomposition point. The optimum operating temperature for specific baths may vary somewhat, but usually temperatures about 5-20° F. above the melting point and below about 170° F. are satisfactory when the complexing agent is diethyl ether. The current density may vary over wide ranges. For example, the lower limit is largely practical in nature and may be 0.1-1 ampere/sq. ft., while the upper limit may be 50-150 amperes/sq. ft. or higher.

Excellent plate may be produced from the above described baths but the resistivity is often of the order of about 1200-1300 ohm-centimeters and thus the power consumption is high. It has been further discovered that the resistivity may be reduced by dissolving in the baths at least one soluble ionizable compound such as quaternary ammonium compounds, amine salts, and nonoxygen-containing mineral acids and salts thereof in an amount to lower the initial resistivity. By this method, often the initial resistivity of 1200-1300 ohm-centimeters may be reduced to about 600-700 ohm-centimeters or lower. It is usually not possible to further reduce the resistivity below this level due to the relatively low solubility of such substances in the baths, which may be about 0.5% to 5-10%. In most instances, the ionizable compound is dissolved in the bath to the extent of its solubility, but smaller amounts may reduce the resistivity somewhat.

A wide variety of compounds of the foregoing types may be dissolved in the plating baths of the present invention. Examples of quaternary ammonium compounds include quaternary amine salts and pyridinium compounds wherein the organic radicals attached to the nitrogen atom may contain 1-8 to 20 carbon atoms. Specific examples include tetramethyl, tetraethyl, tetrapropyl, tetrabutyl, tetraamyl, tetrahexyl, tetraoctyl and higher ammonium halides or other suitable salts of nonoxygen-containing mineral acids. The organic radicals attached to the nitrogen atom may or may not be the same. For example, dodecyl trimethyl ammonium chloride and equivalent mixed quaternary ammonium salts may be used. Pyridinium compounds include methyl, propyl, amyl, octyl and higher alkyl pyridinium nonoxygen-containing mineral acid salts wherein the alkyl radical contains, for example, 1-8 to 20 carbon atoms. The nonoxygen-containing mineral acid salts of the pyridinium compounds include halides such as chlorides, bromides, etc. Inorganic salts include alkali metal nonoxygen-containing mineral acid salts, alkaline earth metal nonoxygen-containing mineral acid salts, and

nonoxygen-containing mineral acid salts in general which are soluble in an amount to reduce the resistivity of the bath. Specific examples include the halides of the foregoing groups of metals and especially the chlorides and bromides. Lithium chloride is usually preferred.

The amine salts may be derived from amines containing 1 to 3 organic radicals attached to the nitrogen atom having 1-8 to 20 carbon atoms. Preferably, the organic radicals are alkyl and the salts are formed from a nonoxygen-containing mineral acid such as hydrochloric, hydrobromic, etc. Still other ionizable compounds include nonoxygen-containing mineral acids such as the hydrogen halides and alkali or alkaline earth metal salts thereof, and especially organic derivatives wherein at least one ionizable hydrogen atom of the mineral acid has been replaced by an organic radical containing, for example, 1-8 to 20 carbon atoms. The resultant organic compound containing a mineral acid group or the alkali or alkaline earth metal salt thereof may be dissolved in the bath to some extent, and the resistivity is reduced due to the ionization of the mineral acid substituent.

Ionizable compounds of the above types may reduce the initial resistivity of the basic bath to about 600-700 ohm-centimeters. The resultant bath may be used, as may the basic bath, for the electrodeposition of very satisfactory electrodeposits of a coating metal such as aluminum, aluminum alloys, or other metals mentioned herein. However, the power consumption is higher than ideal in commercial installations and it is usually desirable that the resistivity be reduced still lower.

In accordance with another variant of the invention, it has been discovered that the resistivity of the basic bath may be reduced a still greater extent by means of a difunctional compound having a complexing function for the aluminum halohydride and/or aluminum halide constituents of the bath and, in addition, thereto, an ionizable substituent. Since the difunctional compound is both a complexing agent and an ionizable compound and complexes the aluminum halohydride and/or aluminum halide, it is soluble in the bath in large amounts and the ionizable substituent is likewise solubilized in large amounts. Due to the increase in the concentration of the ionizable substituent and the availability of additional ions for carrying the current, the initial resistivity of the basic bath may be reduced markedly to about 70 ohm-centimeters or lower. This may be accomplished without a decrease in the flash point and the bath remains non-combustible at the operating temperature.

The difunctional compounds may contain the same types of complexing groups that are present in the simple complexing agents previously described and, similarly, the same types of ionizable groups that are present in the ionizable compounds previously described. Thus, the difunctional compound may be considered to be a complexing agent of the types previously described which is also an ionizable compound selected from the group consisting of quaternary ammonium compounds, amine salts, and organic compounds containing a nonoxygen-containing mineral acid group and salts thereof as defined herein.

Usually it is preferred that about 33-66 mole percent of the total amount of complexing agent contain an ionizable substituent. However, in some instances amounts as low as 15-25 mole percent and up to 75-85 mole percent may be used. Even 1 mole percent improves the conductivity.

Ethers are the preferred complexing agents and quaternary amine salts are the preferred ionizable compounds. In instances where both the ether linkage and quaternary amine group are present in the same molecule, the compounds may be of the following classes:



where R and R'' are monovalent organic radicals containing up to about 20 carbon atoms and preferably 1-8 carbon atoms, R' is a divalent organic radical containing up to about 20 carbon atoms and preferably 1-8 carbon atoms, and Y is a nonoxygen-containing mineral acid residue such as halogen, etc. In most instances, alkyl or alkylene radicals containing 1-8 carbon atoms are preferred.

Of the above types of compounds, ethoxyethyltrimethyl ammonium chloride is preferred. Other specific ethers containing quaternary ammonium groups which may be used are methoxymethyltrimethyl ammonium halides such as the chloride, bis(2-dimethylaminoethyl) ether dimethhalides such as the chloride, N-ethyl-N-methyl morpholinium halides such as the iodide or chloride and 2-ethoxyethyltriethyl ammonium halides such as the iodide or chloride.

In instances where the plating bath contains aluminum chloride, aluminum dichlorohydride, ethyl ether, and ethoxyethyltrimethyl ammonium chloride, the following compositions are especially useful:

|                                             | Broad Range (Moles) | Preferred Amount (Moles) |
|---------------------------------------------|---------------------|--------------------------|
| Aluminum Chloride.....                      | 0-4                 | 3.8                      |
| Aluminum Dichlorohydride.....               | 6-2                 | 2.0                      |
| Diethyl Ether.....                          | 2-4                 | 3.8                      |
| Ethoxyethyltrimethyl Ammonium Chloride..... | 4-2                 | 2.0                      |

The preferred bath above defined has a melting point of approximately 80-90° F. The operating temperature range for the electrodeposition of aluminum or aluminum alloy therefrom is above the melting point and preferably below about 160-170° F. Best results are usually obtained at an operating temperature of about 115-135° F.

The lower limit on the current density to be employed is practical in nature, and current densities as low as 0.1 to 1 ampere/sq. ft. may be used. Current densities as high as 150-300 amperes/sq. ft. may be used with the preferred baths, and often as high as 1000 amperes/sq. ft. in instances where the preferred additives for reducing resistivity are used. Generally, when additives for reducing resistivity are not present, current densities up to 50-150 amperes sq. ft. will give better results. Special plating conditions may be used if desired such as pulse current, polarity reverse current, etc., or the plating may be conducted with vigorous agitation, rotating or rapidly moving cathodes, etc.

The coating metal may be supplied to the plating bath by any suitable convenient means such as by addition of a soluble salt of the coating metal, by soluble anodes, or by auxiliary anodes. In the specification and claims, it is understood that an electroplating bath of the invention contains the metal or metals to be electrodeposited on the substrate in a form that may be electroplated therefrom. When an aluminum-containing coating is electrodeposited, preferably aluminum anodes or aluminum alloy anodes are immersed in the bath in the usual manner. Other metals that may be electrodeposited include titanium, zirconium, vanadium, columbium, beryllium, molybdenum, tungsten, chromium, tantalum, magnesium, manganese, nickel, cobalt, iron, copper, and alloys thereof with or without aluminum. Preferably, in instances where aluminum is being deposited and iron is present in the bath, the concentration of iron is maintained below 0.2% by weight, and preferably between 0.01 and 0.02%.

The thickness of the aluminum plate may vary over wide ranges. Usually, for strip plating thin deposits are preferred such as  $15 \times 10^{-6}$  to  $90 \times 10^{-6}$  inch. However, much heavier deposits are possible such as up to several thousandths of an inch, e.g.,  $5 \times 10^{-3}$  to  $15 \times 10^{-3}$  inch, or even up to  $\frac{1}{8}$  to  $\frac{1}{2}$  inch. It is also possible to use the plating bath of the present invention for electroforming.

When so used, preferably additives are present which tend to reduce treeing.  $\beta\beta'$  dichloroethyl ether may be used as an addition agent to improve the smoothness and hardness of the plating, regardless of whether electroplating items such as steel strip or in electroforming. This ether may be added in an amount sufficient to constitute 4-8% by volume of the bath, but smaller or larger amounts may be added in some instances.

The coating metals described herein may be electrodeposited on any suitable conductive substrate. Preferably, the substrate is ferrous metal in the form of strip, wire, or other metal articles. Still other metallic substrates may be used if desired, as may normally non-conductive substrates which have been treated with a conductor to render them conductive for purposes of the present invention. Such materials are well known and the selection of a specific conductive substrate for practicing the present invention is within the skill of the art.

It is preferred that metallic substrates such as ferrous metal be activated or etched prior to the electrodeposition of aluminum. This may be done by any suitable method known to the art, such as by treatment with hydrogen chloride gas in a carrier gas. In one preferred method, the metal is dipped in a long chain fatty acid such as oleic, rinsed in an ether solution of aluminum halohydride, and then plated. In another preferred method, the metal is cleaned mechanically in an anhydrous atmosphere to provide a fresh, clean surface. For best results the foregoing treatments should be effected under

Preferably the free solvent content of the bath is maintained at a level sufficiently low to provide an ignition point as determined by ASTM D-286-58T that is above the operating temperature of the bath and usually above 500° F. Also, the bath should be prepared under anhydrous conditions and maintained substantially anhydrous throughout its life. For instance, the bath should not contain the decomposition products of over about 1% by weight of water when such water has been deactivated by treatment of the bath with a metal hydride in an amount to provide at least about two gram atoms of active hydrogen per mole of water. Additionally, the bath should not contain over about 0.02-0.03% of water which has not been deactivated by addition of a metal hydride as at water concentrations greater than this the bath is detrimentally affected. Within the above limits, a bath containing water may be restored to its former condition and excellent plate again obtained by addition of the metal hydride in the prescribed amounts.

As disclosed in my copending application Serial No. 159,447, filed December 14, 1961, now Patent 3,214,228 for Process for the Deposition of Metals and the Resultant Products, the halohydride-containing compositions of the invention may be used in the electroless deposition of metallic aluminum-containing material on a wide variety of bases or substrates including metals such as ferrous metal, brass, copper, etc., and nonmetallic substrates such as wood, composition board, plastics, etc. This may be conveniently accomplished by decomposing an aluminum halide-containing composition of the invention to produce metallic aluminum in intimate contact with the substrate on which the aluminum is to be deposited. The decomposition may be effected by heating a body of the composition from a lower temperature up to or above the decomposition temperature while in intimate contact with the substrate, or the substrate may be heated above the decomposition temperature and contacted with the composition.

Where the melting point of a specific bath composition is undesirably high, a noncombustible liquid or low melting point diluent which is not detrimental to the electrodeposition of a metal therefrom may be added to reduce the melting point. Preferably, the diluent is inert with respect to the bath at the temperatures encountered.

The foregoing detailed description and the following specific examples are for purposes of illustration only

5

10

15

20

25

30

35

40

45

50

55

60

65

70

75

and are not limiting to the spirit or scope of the appended claims.

#### Example I

The monoetherate of  $\text{AlHCl}_2$  was prepared by treating aluminum chloride in ether solution with lithium aluminum hydride in the calculated amount to form  $\text{AlHCl}_2$ . Excess or solvent ether was evaporated from the resultant product, and the ether content further reduced to the monoetherate of  $\text{AlHCl}_2$  by aeration with dry gaseous nitrogen.

The resultant monoetherate of  $\text{AlHCl}_2$  was heated to the molten condition, aluminum anodes immersed therein, and the resultant bath used for plating steel panels at 30 amperes/sq. ft. at temperatures of 82° F. and 115° F. A thickness of about 0.03 mil of aluminum was deposited on the steel panels in the form of an adherent white mat plate which could be roll brightened.

The resistivity of the bath was determined and found to be 309 ohm-centimeters at 100° F. The bath was tested and found to be noncombustible at the plating temperatures.

#### Example II

A plating bath was prepared by dissolving aluminum chloride in diethyl ether, and then treating the solution with lithium aluminum hydride in the calculated amount to produce 2 moles of  $\text{AlHCl}_2$  for each 3.8 moles of aluminum chloride remaining in the ether solution. Excess ether was evaporated from the resultant product to produce the monoetherates of the  $\text{AlHCl}_2$  and  $\text{AlCl}_3$ .

The above prepared composition contained 2 moles of aluminum dichlorohydride etherate for each 3.8 moles of aluminum chloride etherate. The composition was used as a plating bath for electrodepositing aluminum on ferrous metal panels at 30 amperes/sq. ft. and at a temperature of 115° F. Aluminum anodes were immersed in the plating bath during the electrodeposition.

The aluminum plated out on the ferrous metal panels in the form of a white mat coating and was pleasing in appearance, adherent, and could be obtained in any desired thickness. The white mat plate could be roll brightened, or other forms of brightening could be used.

If desired, the corresponding aluminum bromide salt may be prepared by using aluminum bromide as the starting material. The resultant bath could be used for the electrodeposition of aluminum.

#### Example III

The new compound 2-ethoxyethyltrimethyl ammonium chloride was prepared by heating 54.5 grams (0.5 mole) of 2-chloroethyl ethyl ether and 120 grams (0.55 mole) of 25% triethyl amine in methanol in a steel bomb at 125° C. for 15 hours. Thereafter, the mixture was evaporated to a syrup on a rotating evaporator at 70° C., dissolved in ethyl alcohol (100 ml.) and evaporated to dryness. The product was dispersed in acetone, filtered with suction while preventing contact with moisture, and then dried in vacuum at 80° C. The resultant product was 70.1 grams of a white solid (83.5% of the theoretical yield) which was identified as being 2-ethoxyethyltrimethyl ammonium chloride.

The above procedure was modified somewhat by dissolving 123 grams (1.13 moles) of 2-chloroethyl ethyl ether and 307 grams (1.3 moles) of 25% trimethyl amine in methanol, and heating in a glass bottle at 70° C. for 15 hours. Thereafter, the product was evaporated to dryness using a rotating evaporator at 70° C., the product dispersed in ethyl alcohol (200 ml.) and evaporated to dryness, repeated, slurried with acetone, filtered with suction, washed with acetone and pentane, and then dried in vacuum at 80° C. overnight.

The resultant product was 152.1 grams of off-white crystalline solid (80.2% of the theoretical yield), and this likewise was identified as being 2-ethoxyethyltrimethyl ammonium chloride.

*Example IV*

Lithium hydride was added to a diethyl ether solution of aluminum chloride in the calculated amount to produce 2 moles of aluminum dichlorohydride for each 3.8 moles of aluminum chloride remaining in the solution. The resultant ether solution contained excess solvent or free ether, which was evaporated by heating to the boiling point of the bath.

With continued evaporation, the boiling point of the bath gradually rose until a temperature of 160° F. was reached. At this point, the bath was cooled and dry nitrogen was bubbled through the bath at about room temperature to thereby strip the remaining ether out of the bath and produce a mixture of the monoetherate of aluminum dichlorohydride and the monoetherate of aluminum chloride. At this point, the flash point of the bath was about 200-215° F., and no further rise of the flash point was noted with continued stripping with the nitrogen. The resultant bath had a melting point of about 90° F., and was used as a plating bath for the electrodeposition of aluminum.

Aluminum anodes were immersed in the bath and aluminum electrodeposited on steel panels at temperatures from slightly above the melting point up to a temperature just below the decomposition point (about 160-175° F.). The preferred temperature range was found to be 115-135° F. Current densities between 0.1 ampere/sq. ft. and 150 amperes/sq. ft., and preferably 1-100 amperes/sq. ft. could be used to produce white mat aluminum plate of good quality.

The resistivity of the above bath was about 1200-1300 ohm-centimeters and it was noncombustible at the operating temperatures.

*Example V*

A plating bath is prepared in accordance with the procedure of Example IV, the bath divided into a number of portions and then each of the portions is saturated with one of a number of ionizable compounds. The bath had a resistivity of about 1200-1300 ohm-centimeters. Ionizable compounds for addition to different portions of the bath include tetramethyl ammonium chloride, dodecyltrimethyl ammonium chloride, amine salts, and organic compounds containing a nonoxygen-containing mineral acid function and salts thereof.

The addition of the above compounds reduces the resistivity of the bath. The most effective are the quaternary ammonium compounds, which lowered the resistivity from about 1200-1300 ohm-centimeters to approximately 600-700 ohm-centimeters.

The resultant bath was as satisfactory as the bath of Example IV for the electrodeposition of aluminum. In addition, the power requirements were lower due to the lower resistivity.

*Example VI*

A plating bath was prepared from the following:

|                                                | Moles |
|------------------------------------------------|-------|
| AlCl <sub>3</sub> -----                        | 3.8   |
| AlHCl <sub>2</sub> -----                       | 2.0   |
| Ethyl ether -----                              | 3.8   |
| 2-ethoxyethyltrimethyl ammonium chloride ----- | 2     |

The above composition was heated to the melting point. The resultant bath was essentially a monoetherate of aluminum chloride plus a monoetherate of aluminum chlorohydride, of which 2 moles of the ether is 2-ethoxyethyltrimethyl ammonium chloride.

The above bath was noninflammable and had a resistivity of approximately 70 ohm-centimeters. When used for the electrodeposition of aluminum on steel panels, the bath produced excellent mat aluminum plate at current densities up to 300 amperes/sq. ft. The preferred temperature of electrodeposition was 115-135° F. Aluminum deposits of any desired thickness could be produced, and the bath could be used for electroforming.

What is claimed is:

1. A process for electrodepositing a metallic material on an electrically conductive substrate comprising subjecting at least a portion of the substrate as a cathode to the action of an electrolyzing electric current while immersed in a bath consisting essentially of an organic complex of an aluminum halohydride, the bath being noncombustible at the operating temperature and substantially free of an uncombined solvent for the organic complex of the aluminum halohydride.
2. A process for electrodepositing a metallic material on an electrically conductive substrate comprising subjecting at least a portion of the substrate as a cathode to the action of an electrolyzing electric current while immersed in a bath consisting essentially of an organic complex of aluminum halide and an organic complex of an aluminum halohydride, the bath being noncombustible at the operating temperature and substantially free of an uncombined solvent for the organic complex of the aluminum halide and the organic complex of the aluminum halohydride.
3. A process for electrodepositing a metallic material on an electrically conductive substrate comprising subjecting at least a portion of the substrate as a cathode to the action of an electrolyzing electric current while immersed in a bath consisting essentially of an organic complex of an aluminum halohydride, the bath being noncombustible at the operating temperature and having dissolved therein at least one soluble ionizable compound selected from the group consisting of quaternary ammonium compounds, amine salts, and nonoxygen-containing mineral acids and salts thereof.
4. A process for electrodepositing an aluminum containing material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen selected from the group consisting of chlorine, bromine and mixtures thereof, the bath being noncombustible at the operating temperature and having dissolved therein at least one soluble ionizable compound selected from the group consisting of quaternary ammonium compounds, amine salts, and nonoxygen-containing mineral acids and salts thereof.
5. A process for electrodepositing an aluminum containing material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen selected from the group consisting of chlorine, bromine and mixtures thereof, the bath being noncombustible at the operating temperature and substantially free of an uncombined solvent for the etherate of the aluminum halide and the etherate of the aluminum halohydride and having a mole ratio of AlH<sub>3</sub> to AlCl<sub>3</sub> between about 1:0.5 and 1:22.
6. A process for electrodepositing an aluminum-containing material on an electrically conductive substrate comprising subjecting at least a portion of the substrate as a cathode to the action of an electrolyzing electric current while immersed in a bath consisting essentially of a monoetherate of aluminum chloride and a monoetherate of an aluminum chlorohydride, the monoetherates being formed from at least one ether having organic radicals attached to the oxygen atom containing 1-8 inclusive carbon atoms, the bath being noncombustible at the operating temperature and having a mole ratio of AlH<sub>3</sub> to AlCl<sub>3</sub> between about 1:2 and 1:11.
7. A process for electrodepositing an aluminum-containing material on an electrically conductive substrate comprising subjecting at least a portion of the substrate as a cathode to the action of an electrolyzing electric current

while immersed in a bath consisting essentially of a monoetherate of aluminum chloride and a monoetherate of an aluminum chlorohydride, the ether forming the etherates comprising diethyl ether, the bath having a flash point not less than about 200° F. and a mole ratio of  $\text{AlH}_3$  to  $\text{AlCl}_3$  between about 1:2 and 1:11.

8. A process for electrodepositing an aluminum-containing material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen selected from the group consisting of chlorine, bromine and mixtures thereof and being formed from at least one ether having organic radicals attached to the oxygen atom containing 1-8 inclusive carbon atoms, the bath having a mole ratio of  $\text{AlH}_3$  to  $\text{AlCl}_3$  between about 1:0.5 and 1:22, the bath being noncombustible at the operating temperature and having dissolved therein at least one soluble ionizable compound selected from the group consisting of quaternary ammonium compounds, amine salts, and nonoxygen-containing mineral acids and salts thereof.

9. The process of claim 8 wherein the etherates are monoetherates and the ionizable compound dissolved in the bath is an alkali metal halide.

10. A process for electrodepositing an aluminum-containing material on an electrically conductive substrate comprising subjecting at least a portion of the substrate as a cathode to the action of an electrolyzing electric current while immersed in a bath consisting essentially of a monoetherate of aluminum chloride and a monoetherate of an aluminum chlorohydride, the ether forming the etherates comprising diethylether, the bath having a flash point not less than about 200° F. and a mole ratio of  $\text{AlH}_3$  to  $\text{AlCl}_3$  between about 1:2 and 1:11, and the bath having dissolved therein at least one soluble ionizable compound selected from the group consisting of quaternary ammonium compounds, amine salts, and nonoxygen-containing mineral acids and salts thereof.

11. A process for electrodepositing a metallic material on an electrically conductive substrate comprising subjecting at least a portion of the substrate as a cathode to the action of an electrolyzing electric current while immersed in a bath consisting essentially of an organic complex of an aluminum halohydride, the bath being noncombustible at the operating temperature and the complexing agent forming the complex comprising at least one ionizable compound which is also a Lewis base selected from the group consisting of quaternary ammonium compounds, amine salts, and organic compounds containing a nonoxygen-containing mineral acid group and salts thereof.

12. A process for electrodepositing a metallic material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen selected from the group consisting of chlorine, bromine and mixtures thereof the bath being noncombustible at the operating temperature and containing an etherate formed at least in part from an ionizable compound selected from the group consisting of quaternary ammonium compounds containing an ether linkage, amine salts containing an ether linkage, and ethers containing a nonoxygen-containing mineral acid group and salts thereof.

13. A process for electrodepositing an aluminum-containing material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen

5 selected from the group consisting of chlorine, bromine and mixtures thereof, the bath having a mole ratio of  $\text{AlH}_3$  to  $\text{AlCl}_3$  between about 1:05 and 1:22, the bath being noncombustible at the operating temperature and containing an etherate formed at least in part from a quaternary ammonium compound having an ether linkage.

14. A process for electrodepositing a metallic material on electrically conductive substrate comprising subjecting at least a portion of the substrate as a cathode to the action of an electrolyzing electric current while immersed in a bath consisting essentially of an etherate of an aluminum halohydride, the bath being noncombustible at the operating temperature and the ether forming the etherate comprising ethoxyethyltrimethyl ammonium chloride.

15. A process for electrodepositing an aluminum-containing material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen selected from the group consisting of chlorine, bromine and mixtures thereof, the bath being noncombustible at the operating temperature and containing an etherate formed at least in part from ethoxyethyltrimethyl ammonium chloride.

16. A process for electrodepositing an aluminum-containing material on an electrically conductive substrate comprising subjecting at least a portion of the substrate as a cathode to the action of an electrolyzing electric current while immersed in a bath consisting essentially of an etherate of aluminum halide and an etherate of an aluminum halohydride, the etherates containing halogen selected from the group consisting of chlorine, bromine and mixtures thereof, the bath having a mole ratio of  $\text{AlH}_3$  to  $\text{AlCl}_3$  between about 1:0.5 and 1:22, the bath being noncombustible at the operating temperature and containing an etherate formed at least in part from ethoxyethyltrimethyl ammonium chloride.

17. A process for electrodepositing an aluminum-containing material on an electrically conductive substrate comprising subjecting at least a portion of the substrate as a cathode to the action of an electrolyzing electric current while immersed in a bath consisting essentially of a monoetherate of aluminum chloride and a monoetherate of an aluminum chlorohydride, the ether forming the etherates comprising diethyl ether and ethoxyethyltrimethyl ammonium chloride, the bath having a flash point not less than about 200° F. and a mole ratio of  $\text{AlH}_3$  to  $\text{AlCl}_3$  between about 1:2 and 1:11.

18. A bath for electrodepositing a metallic material consisting essentially of an organic complex of an aluminum halohydride, the bath being noncombustible at the operating temperature and having dissolved therein at least one soluble ionizable compound selected from the group consisting of quaternary ammonium compounds, amine salts, and nonoxygen-containing mineral acids and salts thereof.

19. A bath for electrodepositing a metallic material consisting essentially of an etherate of aluminum halide and an etherate of an aluminum halohydride, the etherates containing halogen selected from the group consisting of chlorine, bromine and mixtures thereof, the bath being noncombustible at the operating temperature and having dissolved therein at least one soluble ionizable compound selected from the group consisting of quaternary ammonium compounds, amine salts, and nonoxygen-containing mineral acids and salts thereof.

20. A bath for electrodepositing a metallic material consisting essentially of an etherate of aluminum halide and an etherate of an aluminum halohydride, the etherates containing halogen selected from the group consisting of chlorine, bromine and mixtures thereof and being formed from at least one ether having organic radicals attached to the oxygen atom containing 1-8 inclusive carbon atoms,

the bath having a mole ratio of  $\text{AlH}_3$  to  $\text{AlCl}_3$  between about 1:0.5 and 1:22, the bath being noncombustible at the operating temperature and having dissolved therein at least one soluble ionizable compound selected from the group consisting of quaternary ammonium compounds, amine salts, and nonoxygen-containing mineral acids and salts thereof.

21. A bath for electrodepositing a metallic material consisting essentially of a monoetherate of aluminum chloride and a monoetherate of an aluminum chlorohydride, the ether forming the etherates comprising diethylether, the bath having a flash point not less than about 200° F. and a mole ratio of  $\text{AlH}_3$  to  $\text{AlCl}_3$  between about 1:2 and 1:11, and the bath having dissolved therein at least one soluble ionizable compound selected from the group consisting of quaternary ammonium compounds, amine salts, and nonoxygen-containing mineral acids and salts thereof.

22. A bath for electrodepositing a metallic material consisting essentially of an organic complex of an aluminum halohydride, the bath being noncombustible at the operating temperature and the complexing agent forming the complex comprising at least one ionizable compound which is also a Lewis base selected from the group consisting of quaternary ammonium compounds, amine salts, and organic compounds containing a mineral acid group and salts thereof.

23. A bath for electrodepositing a metallic material consisting essentially of an etherate of aluminum halide and an etherate of an aluminum halohydride, the etherates containing halogen selected from the group consisting of chlorine, bromine and mixtures thereof, the bath being noncombustible at the operating temperature and containing an etherate formed at least in part from an ionizable compound selected from the group consisting of quaternary ammonium compounds containing an ether linkage, amine salts containing an ether linkage, and ethers containing a nonoxygen-containing mineral acid group and salts thereof.

5 24. A bath for electrodepositing a metallic material consisting essentially of an etherate of aluminum halide and an etherate of an aluminum halohydride, the etherates containing halogen selected from the group consisting of chlorine, bromine and mixtures thereof, the bath having a mole ratio of  $\text{AlH}_3$  to  $\text{AlCl}_3$  between about 1:0.5 and 1:22, the bath being noncombustible at the operating temperature and containing an etherate formed at least in part from a quaternary ammonium compound having an ether linkage.

10 25. A bath for electrodepositing a metallic material consisting essentially of a monoetherate of aluminum chloride and a monoetherate of an aluminum chlorohydride, the ether forming the etherates comprising diethyl ether and ethoxyethyltrimethyl ammonium chloride, the bath having a flash point not less than about 200° F. and a mole ratio of  $\text{AlH}_3$  to  $\text{AlCl}_3$  between about 1:2 and 1:11.

#### References Cited by the Examiner

##### UNITED STATES PATENTS

|           |         |                       |           |
|-----------|---------|-----------------------|-----------|
| 1,939,397 | 12/1933 | Keyes et al. -----    | 204—14    |
| 2,446,349 | 8/1948  | Wier et al. -----     | 204—14    |
| 2,651,608 | 9/1953  | Brenner et al. -----  | 204—14    |
| 2,692,850 | 10/1954 | Safranek et al. ----- | 204—39    |
| 2,708,207 | 5/1955  | Girod -----           | 260—567.6 |
| 2,727,923 | 12/1955 | Husted -----          | 260—567.6 |
| 2,849,349 | 8/1958  | Ziegler et al. -----  | 204—14    |
| 2,992,248 | 7/1961  | Pearson -----         | 23—14     |
| 3,007,854 | 11/1961 | Smith et al. -----    | 204—39    |

##### OTHER REFERENCES

Brenner et al., "A Hydride Bath for the Electrodeposition of Aluminum," Journal of the Electrochemical Society, vol. 99, No. 6, June 1952, pages 234—244.

JOHN H. MACK, *Primary Examiner.*

JOSEPH REBOLD, JOHN R. SPECK, *Examiners.*

R. GOOCH, R. K. MIHALEK, *Assistant Examiners.*